# EUROPEAN PATENT SPECIFICATION

(11) **EP 2 132 156 B1**
(45) Date of publication and mention of the grant of the patent: **27.11.2013**
(21) Application number: 08726928.8
(22) Date of filing: 18.03.2008
(51) Int. Cl.: C07C 2/64

(54) **ALKYLAROMATIC LUBRICANT FLUIDS**
ALKYLAROMATISCHE SCHMIERFLÜSSIGKEITEN
LIQUIDES LUBRIFIANTS ALKYLAROMATIQUES

(30) Priority: 20.03.2007 US 919018 P; 14.03.2008 US 75948
(43) Date of publication of application: 16.12.2009
(73) Proprietor: ExxonMobil Research and Engineering Company, Annandale, NJ 08801-0900 (US)
(72) Inventor: YOON, Beth, A., Pennington, NJ 08534 (US); WU, Margaret, M., Skillman, NJ 08558 (US); ELIA, Christine, N., Bridgewater, NJ 08807 (US)
(74) Representative: Mareschal, Anne
(86) International application number: PCT/US2008/003518
(87) International publication number: WO 2008/127534

(56) References cited:
- EP-A1- 0 305 114
- WO-A1-2005/042448
- US-A- 4 871 476
- US-A- 5 132 477
- US-A- 5 625 105
- US-A1- 2003 149 203
- US-A1- 2004 018 944

## Description

### FIELD

The present disclosure relates to novel alkylaromatic compositions useful as lubricant basestocks and additives. More particularly, the compositions of the present disclosure are quaternary-substituted alkylaromatic compositions that have improved thermo- and oxidative stability prepared by alkylating aromatics with vinylidene-containing olefins. The present disclosure also relates to processes for producing alkylaromatic compositions that employ acidic alkylation catalysts.

### BACKGROUND

A lubricant is a substance capable of reducing friction, heat and wear when introduced as a film between solid surfaces. Efforts to improve upon the performance of mineral oil based lubricants have been the focus of important research and development activities in the petrochemical industry for over 50 years. Maintenance of friction reducing properties, extended useful life in terms of thermal and oxidative stability and wear protection, improved viscosity index and pour point equal to or better than mineral oil are performance areas where research and development activities have occurred. These efforts have led to the introduction of a number of synthetic fluids including polyalpha-olefin (PAO) synthetics primarily made by oligomerization of alpha-olefins or 1-alkenes. Synthetic fluids is a term that can describe materials useful as lubricants, heat transfer agents, and corrosion inhibition among other uses. PAO synthetic fluids compositions are saturated hydrocarbons and thus are less polar than mineral oil based compositions that can contain polar moieties including aromatics. To improve the solvency and dispersancy of PAO type fluids, a polar co-basestock is added to the composition to help dissolve polar additives of the composition and sludge during usage. A polar co-basestock such as ester or alkylaromatics is used in amounts of about 3 to about 50 weight percent of the basestock composition. The polar co-basestock could introduce undesirable side effects such as hydrolytic instability if an ester co-basestock is used or poorer low temperature properties, reduced cleanliness properties if typical alkylaromatic co-basestocks are used. Finished synthetic lubricants are often formulated with additives to enhance their properties for specific applications. Additives that are commonly used can include oxidation inhibitors, dispersants, detergents, rust inhibitors, antiwear agents, extreme pressure agents, metal passivators, pour point depressants, viscosity index (VI) improvers, and the like. Thus formulated fluids are compositions comprising a number of components, the largest volume component being the fluid basestock. Adding to the complexity of formulating lubricating oils is the trend to ever higher oil performance standards dictated by the increasing complexity of newer equipment and engines. There is a continuing need to improve the suite of properties of the fluid basestock to provide improved performance of the formulated products in all areas required including thermal and oxidative stability.

Alkylaromatic compounds have been known for many years. For example, US Patent No. 6,491,809 (Briot et al.) discloses the alkylation of aromatic compounds (e.g., benzene, toluene, cumene) by alkylating agents (e.g., olefins, alcohol, halides) for producing aromatic monoalkyls whose grafted aliphatic chain comprises a carbon number that is selected from 2 to 20 carbons. US Patent No. 6,429,345 (Joly et al.) discloses a process for producing at least one compound selected from 2-, 3-, 4-, 5- and 6-phenylalkanes by alkylating benzene using at least one olefin containing at least 9 carbon atoms per molecule, in the presence of a catalyst comprising at least one zeolite with structure type EUO, at least partially in its acid form and at least one matrix. US Patent No. 5,254,274 (Ho et al.) discloses alkylating aromatic compounds with C₂₀-C₁₃₀₀ olefinic oligomers using an acidic alkylation catalyst to produce alkylated aromatic products, usually alkylaromatic hydrocarbons. Additional discussions of alkylaromatics and other synthetic lubricants can be found in L.R Rudnick and R.L. Shubkin's Synthetic Lubricants and High-Performance Functional Fluids, Marcel Dekker, Inc., NY (1999).

PAOs can be produced by reacting an olefin feed in the presence of a catalyst such as AlCl₃, BF₃, or promoted BF₃. Processes for the production of PAOs are disclosed, for example, in the following patents: U.S, Pat. Nos. 3,149,178; 3,382,291; 3,742,082; 3,769,363; 3,780,128; 4,172,855; and 4,956,122. Novel PAO lubricant compositions in which little double bond isomerization is found has resulted in different classes of high viscosity index PAO (HVI-PAO). In one class of HVI-PAO, reduced chromium catalyst is reacted with an alpha-olefin monomer. Such PAOs are described in U.S. Pat Nos. 4,827,073; 4,827,064; 4,967,032; 4,926,004; and 4,914,254.

Recently patents describe HVI-PAOs compositions prepared by contacting one or more alpha-olefins monomers having 3 to 24 carbons atoms with a transition metal compound, an anion activator and an alkyl aluminum compound. The novel compositions conform to the unique specificity of the HVI-PAO oligomerization reaction in that little double bond isomerization occurs. Such HVI-PAOs are described in PCT Patent Publication Nos. W02007011462 A1 and W02007011832 A1.

Novel compositions of low viscosity PAOs can also be prepared from metallocene catalysts as taught in U.S. Patents 5,688,887 and 6,043,401 and PCT Patent Publication No. WO2007011973 A1. Separation of the low molecular weight material, representing non-lube range molecular weight material, is necessitated to control product volatility and viscosity. As oligomerization conditions are changed to produce the lower viscosity products of lower average molecular weight, the non-lube range dimer or light end fraction increases. The increase in dimer by-product yield represents a substantial economic burden on the overall process to produce useful lower viscosity lubricant in the process.

Accordingly, there is a need for improved processes for the manufacture of the alkylaromatic fluid compositions as well as alkylaromatic fluid compositions that have improved thermal and oxidative stability. There is also a need for novel processes to utilize the by-products from the metallocene process to produce novel synthetic lubricant fluids.

### SUMMARY

The present disclosure relates to an alkylaromatic compositions comprising an aromatic moiety other than unsubstituted naphthalene; and an alkyl moiety having a carbon atom number in the range between 16 to 40, wherein said alkyl moiety is attached to said aromatic moiety such that at least 25 mol% of the benzylic carbons are quaternary.

The present disclosure also includes a process for the preparation of an alkylaromatic compound comprising: contacting at least one an aromatic compound and a mono-olefin having a carbon atom number in the range between 16 to 40 in the presence of an acidic alkylation catalyst under alkylation conditions, wherein at least 50 mol% of the mono-olefin comprises a vinylidenyl structure and thereby producing said alkylaromatic compound having at least 25 mol% of benzylic carbons that are quaternary.

The present disclosure also provides a process for the utilization of the by-product from the metallocene process to produce a novel synthetic lubricant fluid.

Accordingly, the present disclosure provides useful alkylaromatic fluid compositions that have thermal and oxidative stability.

In addition, the present disclosure provides useful lubricant additives from aromatics alkylation by using vinylidene containing low molecular weight olefins as the alkylating agent.

These and other features and attributes of the disclosed alkylaromatic compositions suitable as liquid lubricant compositions or additives and processes for the preparation of the alkylaromatic compositions of the present disclosure and their advantageous applications and/or uses will be apparent from the detailed description which follows.

### DETAILED DESCRIPTION

It has been discovered that a new synthetic basestock with significantly improved lubricating properties can be produced by reacting aromatics with vinylidene-containing olefins. This new base stock may be produced in such a manner such that a significant amount of the alkylated aromatic is quaternary substituted alkylaromatic.

In some embodiments, the mono-olefin may be derived from the non-lubricant of metallocene-catalyzed alpha olefin polymerization process. Monoolefins derived in other manners with a significant amount of vinylidene may also be advantageous.

Also suitable for use in the processes disclosed herein are refinery feedstocks or effluents. Olefins suitable for the preparation of the dimers or mixtures of dimers, trimers and the like contain from about 3 to 20 carbons, such as 1-propylene, 1-butene, 1-hexene, 1-octene, 1-decene, 1-dodecene, 1-tetradecene, and 1-hexadecene or branched olefins such as 4-methyl-1-pentene or mixtures thereof. The mono-olefin is a vinylidene with a carbon atom number less than 30 and may be a mixture of olefins with a significant amount of vinylidenes or trisubstituted olefins. Generally, at least 50 mol% , or at least 55 mol%, or at least 60 mol%, or at least 65 mol%, of the mono-olefin comprises a vinylidenyl structure.

The aromatic compound may be benzene, furan, thiophene, anthracene, phenanthrene, pyrole, indole, benzothiophene, dibenzothiophene, benzofuran, dibenzofuran, phenoxathiin, thianthrene, biphenyl, pyrene, and mixtures thereof, each of which can be optionally substituted.

In further preferred embodiments, the aromatic compound may be toluene, o-, or p-xylene, hydroxyl benzene, alkoxybenzene such as methoxy or ethoxybenzene, thioanisole, diphenylether, diphenylmethane, bisphenol-A, bisphenol sulfide, diphenyl sulfide, methylnaphthalene, methoxynaphthalene, ethoxynaphthalene, methylnaphthal sulfide, ethyl naphthylsulfide, or mixtures thereof. In more preferred embodiments the aromatic compound may be substituted benzene or substituted naphthalene.

### Process and Product

The general process according to the present disclosure is as follows: In the present disclosure, aromatic hydrocarbons, including substituted aromatic hydrocarbons, are alkylated with olefins, containing a significant amount of vinylidene substitution (generally, at least 50 mol% , or at least 55 mol%, or at least 60 mol%, or at least 65 mol%, of the mono-olefin includes vinylidene). These can be from the non-lube range oligomers made during the metallocene-low viscosity alpha olefin polymerization process (reaction A). The olefins used in the alkylation have a significant amount of vinylidene isomers. Other processes to make vinylidene containing olefins are also included within the scope of the present disclosure. The solid state acid catalysts such as zeolites or Friedel Crafts alkylation catalysts such as AlCl₃ or BF₃ are used to catalyze the alkylation. The resulting novel compositions contain a significant amount of quaternary substitution at the benzylic carbon. The compositions exhibit excellent additive solubilizing properties.

### Olefin

For the purpose of preparing alkylaromatic compositions suitable as liquid lubricant compositions or additive of the present disclosure, a thermally and oxidatively stable composition cam be obtained with an alkylaromatic composition with a significant amount of quaternary benzylic carbon atoms and total side chain carbon content between 16 and 40 carbon atoms. For example, selected compositions can be prepared by a high activity zeolite catalyst, a one or two ring aromatic substrate, and a vinylidene olefin that is a by-product from the metallocene-catalyzed alpha-olefin polymerization process. The metallocene-catalyzed PAO process consists of the oligomerization of 1-alkenes in contact with a metallocene type catalyst. A characteristic of the oligomerization reaction from which these vinylidene olefin by-products are produced is the production of mixtures of dialkyl vinylidenic and 1,2 dialkyl or trialkyl mono-olefin oligomers as determined by infrared and NMR analysis. The processes of the present disclosure result in a significant proportion of unhydrogenated dimerized 1-alkene, or alpha-olefin having a vinylidenyl structure as follows:

CH₂=CR₁R₂

where R₁ and R₂ are alkyl groups. Other olefinic compositions having 16 to 40 carbon atoms may be used in the processes of the present disclosure, including olefin oligomers from the acid or metallocene catalyzed oligomerization of alkenes including, for example, propylene and/or butenes and/or pentenes. The presence of vinylidene-containing trimers or higher order are also advantageous. Other processes that form olefinic precursors enriched in vinylidenes can also be used. The reaction of alpha olefins with Ziegler catalysts, such as triisobutyl aluminum, form vinylidene-containing dimers (see CA Patent No. 1,034,967). A process to dimerize alpha olefins with cyclopentadienyl zirconium dichloride or hafnium metallocene, an aluminoxane with or without an trialkyl aluminum cocatalyst, resulted in the selective formation of vinylidene-containing dimers (See US Patents No. 4,658,078 and 5,087,788.

Other mono olefins with the following substitution patterns where R₁, R₂, and R₃ are alkyl groups and R₄ is a hydrogen or an alkyl group, having a total of 16 to 40 carbon atoms may be used to obtain alkylated aromatics with quaternary substitution:

R₁R₂C=CR₃R₄

Generally, at least 50 mol%, or at least 55 mol%, or at least 60 mol%, or at least 65 mol%, of the mono-olefin structure comprises a vinylidenyl structure for the inventive processes disclosed herein.

### Alkylation

Acidic catalysts capable of affecting alkylation of aromatics with olefins include acidic halides (Lewis acids), protonic acids (Bronsted acids), cation exchange resins, Friedel Crafts catalysts, and solid acids including zeolites.

Thus, while numerous acids catalytically promote the alkylation of aromatics with olefins, the present disclosure exhibits that for the purpose of preparing alkylaromatic compositions that are useful as liquid lubricant compositions and additives, high activity zeolites may be effective. Non-limiting exemplary high activity zeolites with surface acidity useful for preparing alkylaromatic compositions that are useful as liquid lubricant compositions and additives include, but are not limited to, MCM-22, MCM-36, MCM-49, MCM-56, ITQ-1, ITQ-3 and any combination thereof. U.S. Patents No. 4,954,325; 5,229,341; 5,236,575; 5,362,697; 6,077,498, and 6,500,404; respectively disclose MCM-22, MCM-36, MCM-49, MCM-56, ITQ-1, ITQ-3.

Non-limiting exemplary Lewis acids include aluminum chloride, aluminum bromide, iron (III) chloride, zinc chloride, boron trifluoride and others. Non-limiting exemplary Bronsted acids include sulfuric acid, nitric acid, hydrochloric acid, hydrofluoric acid, phosphoric acid and others.

Aromatic compounds which may be used in the present disclosure include substituted and unsubstituted one and two ring aromatics and mixtures thereof. Advantageously, the aromatic moiety is at least one chosen from: benzene, toluene, xylenes, and ethylbenzene. Suitable aromatic compounds include, but are not limited to, substituted or unsubstituted benzene, substituted naphthalene, substituted or unsubstituted furan, substituted or unsubstituted thiophene, substituted or unsubstituted anthracene, substituted or unsubstituted phenanthrene, substituted or unsubstituted pyrole, substituted or unsubstituted indole, substituted or unsubstituted benzothiophene, substituted or unsubstituted dibenzothiophene, substituted or unsubstituted benzofuran, substituted or unsubstituted dibenzofuran, substituted or unsubstituted phenoxanthiin, substituted or unsubstituted thianthrene, substituted or unsubstituted biphenyl, substituted or unsubstituted pyrene, bisphenol A, bisphenol sulfide, anisole, thioanisole, diphenyl oxide, diphenyl sulfide, diphenylmethane, their substituted analogs, and mixtures thereof. A substituted naphthalene is a particularly advantageous aromatic compound for the invention compounds and processes disclosed herein.

In further advantageous embodiments, the aromatic compound is benzene, toluene, o-, m- or p-xylene, hydroxybenzene, alkoxybenzene such as methoxy or ethoxybenzene, thioanisole, diphenylether, diphenylmethane, diphenyl sulfide, methylnaphthalene, methoxynaphthalene, ethoxynaphthalene, methylnaphthyl sulfide, ethyl naphthylsulfide, bisphenol-A, bisphenol sulfide or a mixture thereof.

The aromatic compound can be substituted. Suitable substituent groups include alkyl, hydroxy, alkoxy such as methoxy or ethoxy, aroxy such as phenoxy, alkylthio such as methanethio, arylthio such as phenylthio, and aralkyl such as benzyl. Thus, in some advantageous embodiments the aromatic compound is a mono-substituted benzene, for example toluene, or a disubstituted benzene, for example para-, meta- or ortho-xylene.

The amount of catalyst charged to a reactor relative to the olefinic material is 0.1% to 20%, preferably 0.5% to 5%. The mole ratio of aromatic compound e.g., benzene, naphthalene, 1,2,4-trimethylbenzene to olefin starting material is typically between 1:3 and 20:1, preferably 1:2 to 10:1, but depending on the degree of alkylation of the aromatic which is desired, the ratio may be altered accordingly.

Generally, when a zeolite catalytic process is used, the catalyst is charged in a slurry reactor. The reaction may be carried out in a fixed-bed continuous operation wherein the catalyst is in pellet or extruded form and packed in a tubular reactor heated to a desirable temperature. The feed is introduced at a specific weight hourly space velocity (WHSV) ranging from about 0.1 to about 20, preferably from about 0.5 to about 5, to achieve a high conversion. An effective reaction temperature for the preparation of the alkylaromatic compositions is, for example, between room temperature and 350 °C, advantageously between 75 °C and 350 °C. Above 200 °C, the catalyst may affect isomerization, therefore a more advantageous temperature is below 200°C. Preferred reaction conditions include a pressure of from about 1 to about 30 atmospheres, a preferred catalyst charge from about 1 wt% to about 5 wt% in a slurry reactor or a WHSV of about 0.2 to about 4 in a fixed bed continuous operation. The reactants can be in either the vapor phase or the liquid phase and can be neat, i.e., free from intentional admixture or dilution with other material, or they can be brought into contact with the catalyst composition with the aid of carrier gases or diluents such as , for example, hydrogen or nitrogen. The alkylation can be carried out as a batch-type reaction typically employing a closed, pressurized, stirred reactor with an inert gas blanketing system or in a semi-continuous or continuous operation utilizing a fixed or moving bed catalyst system.

Generally, when a Friedel Crafts catalyst is used to affect the alkylation (US Patent 6,071,864), e.g., AlCl₃ or promoted BF₃, process conditions may be carried out a temperature between -30 and 350 °C, typically at a temperature between 30 °C and 90 °C with a pressure typically between 700 and 7000 kPA. As conditions become more severe the Friedel Crafts catalysts causes isomerization of the vinylidene olefin so that the alkylaromatic product will contain a decreased amount of quaternary substituted alkylated aromatic. The alkylation can be carried out as a batch-type reaction typically employing a closed, pressurized, stirred reactor with an inert gas blanketing system or in a semi-continuous or continuous operation.

In the present disclosure, any means of separation that will provide a useful liquid alkylaromatic composition may be utilized. One example of a useful separation scheme following the alkylation of an aromatic is to use an excess of the lighter boiling hydrocarbon, for example, an aromatic and run the alkylation experiment until all of the olefin (vinylidene or other C16-C40 olefin) has been consumed. Then the liquid composition can be separated from the acidic zeolite by ordinary means such as gravity separation or filtration and the unreacted aromatic can be separated from the liquid composition by vacuum distillation and recycled. In the general case of a Friedel Crafts catalyst, the reaction mixture can be quenched with a dilute acid or base solution, washed with water and dried as described in US Patents 5,254,274 and 6,071,864. Although the product of the alkylation has reduced bromine number compared to the starting olefin, mild hydrotreating of residual olefin or dimer co-product is an option.

This will provide the alkylaromatic composition useful as a liquid lubricant or additive.

### Composition

The alkylaromatic products may have the following non-limiting structures: wherein a significant portion of at least one R group is the radical R₂R₃CCH₃ and wherein R has from 16 to 40 carbons, or 16 to 24 carbons and R₂ and R₃ are alkyl groups. For example: The amount of quaternary substituted aromatic was estimated from assignments determined by NMR DEPT experiments. In particular, the alkyl moiety attached to the aromatic moiety may be such that at least 25 mol% of the benzylic carbons are quaternary or such that at least 30 mol% of the benzylic carbons are quaternary, or such that at least 35 mol% of the benzylic carbons are quaternary, or such that at least 40 mol% of the benzylic carbons are quaternary, or such that at least 50 mol% of the benzylic carbons are quaternary, or such that at least 70 mol% of the benzylic carbons are quaternary Other aromatic structures that may be obtained using alternative olefins could result in quaternary substitution such as the general structure: where R₁, R₂, and R₃ are alkyl groups and R₄ is a hydrogen or alkyl group.

Monoalkylated aromatics are the primary product disclosed herein, although multi-substituted aromatic compositions and olefin-olefin products may also be formed. The presence of non-quaternary alkylated aromatics are also present under the condition of isomerization of the olefin or the presence of non-vinylidene olefin reactants.
In the presence of a sufficiently strong acid catalyst, olefins may undergo skeletal rearrangement leading to tertiary carbocations (R₃C+, where R = alkyl) and that tertiary carbocations will alkylate aromatic substrates to produce a composition with a quaternary benzylic carbon adjacent to the aromatic ring. One of the advantages of the present disclosure is that alkylaromatic compositions having quaternary benzylic carbon at sufficiently high levels (defined as at least 25 mol% of the benzylic carbons are quaternary, or such that at least 30 mol% of the benzylic carbons are quaternary, or such that at least 35 mol% of the benzylic carbons are quaternary, or such that at least 40 mol% of the benzylic carbons are quaternary, or such that at least 50 mol% of the benzylic carbons are quaternary, or such that at least 70 mol% of the benzylic carbons are quaternary), such as to provide improved thermal and oxidative stability to the composition. An illustrative example of an alkylaromatic composition from the present disclosure having thermal and oxidative stability is a composition where a significant amount (defined as at least 25 mol% of the benzylic carbons are quaternary. or such that at least 30 mol% of the benzylic carbons are quaternary, or such that at least 35 mol% of the benzylic carbons are quaternary, or such that at least 40 mol% of the benzylic carbons are quaternary, or such that at least 50 mol% of the benzylic carbons are quaternary, or such that at least 70 mol%) of the benzylic carbons are quaternary. The greater the thermal and oxidative stability of the alkylaromatic liquid lubricant composition the lower the requirement for additives to provide required thermal and oxidative stability.

More particularly, alkylaromatic compositions made from an aromatic moiety of unsubstituted naphthalene exhibit an oxidative stability as measured by RBOT of greater than 150, or greater than 155, or greater than 160, or greater than 165 minutes. Alkylaromatic compositions made from an aromatic moiety of toluene exhibit an oxidative stability as measured by RBOT of greater than 30, or greater than 35, or greater than 40, or greater than 45 minutes. In addition, alkylaromatic compositions made from an aromatic moiety of benzene exhibit an oxidative stability as measured by RBOT of greater than 20, or greater than 25, or greater than 30, or greater than 35 minutes. Generally, the greater the degree of branching and greater the chain length of the alkyl moiety yields a lower RBOT (poorer oxidative stability).

Another advantage of the alkylaromatic compositions of the present disclosure is that the pour point of the compositions formed herein is useful. Compositions including alkylaromatic compositions useful as liquid lubricant compositions must be liquid over a wide temperature range. The pour point is the lowest temperature at which a fluid will flow. The lower the pour point of a liquid lubricant composition, the lower the requirement for pour point depressant additives, which is advantageous. In particular, the disclosed alkylaromatic compositions have pour points that are less than or equal to -30°C, or less than or equal to -35°C, or less than or equal to -40°C, or less than or equal to -45°C , or less than or equal to -50°C. Generally, the lower the degree of branching and the greater the chain length of the alkyl moiety yields a higher (less advantageous) pour point.

The following non-limiting examples are illustrative of the various embodiments of the present disclosure and the advantages thereto. It is within the ability of a person of ordinary skill in the art to select other variables from amongst the many known in the art without departing from the scope of the present disclosure. Accordingly, these examples shall serve to further illustrate the present disclosure, not to limit them.

### EXAMPLES

The following examples 1 to 4 are merely supportive and not according to the present invention as defined in the claims.

Examples 5 and 6 are representative of the present invention as defined in the claims.

### Example 1

### Preparation of Alkylated Naphthalene from 1-hexyl-1-deceae and naphthalene

A solution of 200 g 2-hexyl-1-decene 228 g naphthalene, 200 g decane (optional), and 10 g high activity zeolite catalyst (MCM-22) were heated under nitrogen to 125°C for 48 hours. The solution was cooled and filtered. The lubricant-range material was isolated from the mixture by distillation to remove any components boiling below 160°C at 1 millitorr vacuum. Yield: 231 g clear, nearly colorless fluid (74% based on olefin).

### Example 2

### Preparation of Alkylated Naphthalene from 2-octyl-1-dodecene and naphthalene

The procedure was similar to Example 1 except that 250 g 2-octyl-1-dodecene was used. Yield: 268 g clear, bright yellow fluid (74% based on olefin).

### Example 3

### Preparation of Alkylated Naphthalene from 2-octyl-1-dodecene and naphthalene

A solution of 250 g 2-octyl-1-dodecene, 114 g naphthalene, 200 g decane, and 15 g USY catalyst were heated under nitrogen to 175°C for 8 days. The solution was cooled and filtered. The lubricant-range material was isolated from the mixture by distillation to remove any components boiling below 160°C at 1 millitorr vacuum. Yield: 254 g clear, nearly colorless fluid (62% based on olefin).

### Example 4

### Preparation of Alkylated Naphthalene from 2-hexyl-1-decene and naphthalene

17.1 g Naphthalene and 50 mL hexanes were heated to 45 °C under N₂. BF₃.OEt₂ (5.0 mL) was added dropwise to naphthalene mixture. 20.0 g 2-hexyl-1-decene was added dropwise. Reaction was followed by GC. Upon completion (several days) the reaction mixture was quenched with 5% NaOH, washed with water until neutral and dried over sodium sulfate. The lubricant-range material was isolated from the mixture by distillation to remove any components boiling below 160°C at 1 millitorr vacuum. Yield: 21 g clear fluid, 67% based on olefin.

### Example 5

### Preparation of Alkylated Toluene from 2-octyl-1-dodecene and toluene

460 g Toluene, 140 g 2-octyl-1-dodecene, and crushed MCM-49 (4.0 g) were heated to reflux under N₂. The reaction was followed by GC. Upon completion, several days, the reaction mixture was cooled and filtered. The lubricant-range material was isolated from the mixture by distillation to remove any components boiling below 160°C at 1 millitorr vacuum. Yield: 155 g, 67% yield, based on olefin.

### Example 6

### Preparation of Alkylated Benzene from 2-decyl-1-tetradecene and benzene

175 g Benzene, 140 g 2-decyl-1-tetradecene, and crushed MCM-49 (4.0 g) were heated to reflux under N₂. The reaction was followed by GC. Upon completion, several days, the reaction mixture was cooled and filtered. The lubricant-range material was isolated from the mixture by distillation to remove any components boiling below 160°C at 1 millitorr vacuum. Yield: 158 g clear colorless fluid, 91 % yield, based on olefin.

### Comparative Example 1

Comparative Example 1 is a commercial alkylated naphthalene made from 1-hexadecene, naphthalene, and USY catalyst. The majority of isomers are mono-alkylated with a mixture of alpha and beta naphthalene substitution.

### Comparative Example 2

Comparative Example 2 is an alkylated toluene made from C20 internal olefins, toluene, and a Friedel Crafts catalyst. The majority of isomers are mono-alkylated with little quaternary substitution.

**Table 1. Lube Properties of Vinylidene Alkylated Aromatics**

| **Sample Aromatic Group** | **Example 1 Naphthalene** | **Example 2 Naphthalene** | **Example 3 Naphthalene** | **Comparative Example 1 Naphthalene** |
|---|---|---|---|---|
| **Olefin** | **C16 vinylidene** | **C20 vinylidene** | **C20 vinylidene** | **C16 LAO** |
| **Catalyst** | **MCM-22** | **MCM-22** | **USY** | **USY** |
| ***k*V100°C, cSt** | 5.4 | 6.7 | 5.8 | 4.7 |
| ***k*V40°C, cSt** | 40.5 | 49.9 | 38.7 | 29 |
| ***VI*** | 26 | 67 | 69 | 65 |
| **Pour Point, °C** | <-52.7 | <-52.3 | <-54.2 | -39 |
| **Aniline Point, °C** | 37 | 54 | 49 | 34 |
| **B10 oxidation (40h@325F)** | | | | |
| sludge | nil | nil | trace | nil |
| D664-1, mg/gKOH | 0.32 | 0.90 | 2.40 | 2.26 |
| %Viscosity increase | 2 | 15 | 17 | 13 |
| Pb loss, wt% | 0.6 | 4.66 | 13.9 | 14.3 |
| **RBOT, minutes** | 334 | 167 | 86 | 196 |
| **Noack Volatility, % loss** | 13.8 | 5.2 | 8.2 | 12.7 |
| **Quaternary isomer, mol% *(NMR)*** | 70 | 68 | <10 | NA |

The olefins used to synthesize Examples 1-5 have a single branch at the vinylidene carbon and should be identical in structure to vinylidenes made via the metallocene processes. Examples 1, 2, 4, and 5 have 70, 68, and 72 %, respectively, of an isomer with a quaternary carbon alpha to the naphthalene or toluene ring. Example 3 provides an example of an alkylated naphthalene made from a vinylidene which does not have a significant amount of quaternary substitution. The process of using high activity zeolites with acidity on the surface results in higher concentrations of quaternary substitution for bulky vinylidenes. Use of other acidic catalysts such as BF₃ etherate should result in high amounts of quaternary substitution.

Example 4 demonstrates that the BF₃-etherate catalyst has similar selectivity with respect to quaternary substitution:

**Table 2.**

| **Sample** | **Example 4** | **Example 5** | **Example 6** | **Comparative Example 2** |
|---|---|---|---|---|
| **Aromatic Group** | **Naphthalene** | **Toluene** | **Benzene** | **Toluene** |
| **Olefin** | **C16 vinylidene** | **C20 vinylidene** | **C24 Vinylidene** | **C20 olefin** |
| **Catalyst** | **BF₃.Et₂O** | **MCM-49** | **MCM-49** | **Friedel Crafts catalyst** |
| ***k*V100°C, cSt** | 5.2 | 4.0 | 4.4 | 5.2 |
| ***k*V40°C, cSt** | 34.8 | 20.0 | 19.9 | 32.1 |
| ***VI*** | 55 | 72 | 115 | 86 |
| **Pour Point, °C** | -54 | -51 | -30 | -51 |
| **RBOT, minutes** | | 45 | 31 | 20 |
| **Quaternary isomer, mol %** | 72 | 54 | 72 | <5% |

Examples 1 - 4 have much improved pour points (D5985 method) compared to Comparative Example 1, demonstrating that the branching improves pour points.

Example 1 can be directly compared to Comparative Example 1 since both lubricants have the same molecular weight. The RBOT (Rotary Bomb Oxidation Test, D2272 method) is 334 and 196 minutes, respectively, proving that the quaternary carbon causes an improvement in the oxidation stability of the lubricant. Also, the B10 oxidation test (M334 method) demonstrates improvement of the acid number (0.32 vs. 2.26 mg/gKOH, D664-1 method), viscosity increase (2 vs. 13 wt%, D445-5 method) and Pb loss (0.6 vs. 14.3 wt%, D2272 method) during catalytic oxidation of Example 1 vs. Example 3.

Example 2, which is higher in molecular weight and viscosity than Example 1 and Comparative Example 1, also shows improved or equal B10 oxidation properties relative to Comparative Example 1, but not exceeding those of Example 1.

Example 3 demonstrates the loss of resistance to oxidation when there is little quaternary substitution due to isomerization of the vinylidene during the reaction. The USY catalyst was a poor alkylation catalyst for the alkylation of naphthalene with vinylidenes due to the bulk of the olefin. USY catalyst is an excellent alkylation catalyst for conventional alkylated naphthalenes for which linear alpha olefins are used. The result of this isomerization was poorer RBOT results compared to Comparative Examples 1, although their B10 oxidation results were similar.

Example 5 can be directly compared to Comparative Example 2 since both lubricants have the same molecular weight. The RBOT (Rotary Bomb Oxidation Test, D2272 method) is 45 and 20 minutes, respectively, proving that the quaternary carbon causes an improvement in the oxidation stability of the lubricant.

The resulting product was analyzed as summarized below. Oxidation stability was analyzed under the Rotating Bomb Oxidation Test (RBOT) and the B-10 oxidation test. The RBOT test protocol is described in ASTM D2272. The B-10 oxidation test is used to evaluate mineral oil and synthetic lubricants either with or without additives. The evaluation is based on the resistance of the lubricant to oxidation by air under specified conditions as measured by the formation of sludge, the corrosion of a lead specimen, and changes in neutralization number and viscosity. In this method, the sample is placed in a glass oxidation cell together with iron, copper and aluminum catalysts and a weighed lead corrosion specimen. The cell and its contents are placed in a bath maintained at a specified temperature and a measured volume of dried air is bubbled through the sample for the duration of the test. The cell is removed from the bath and the catalyst assembly is removed from the cell. The oil is examined for the presence of sludge, the total acid number (TAN) (ASTM 664), and Kinematic Viscosity (kV) increase at 100° C (ASTM D445). The lead specimen is cleaned and weighed to determine the loss in weight.

### Modeling Example 7

The products described in Examples 1 - 6 were made with a monoolefin with a >95 mol% vinylidene content. The procedure for Example 1 resulted in 70 mol% quaternary isomer for alkylated aromatics. The procedure for Example 5 resulted in 54 mol % quaternary isomer. These numbers were used to calculate the theoretical yield for monoolefins with vinylidene contents of 50 - 65% as shown in Table 3 below.

**Table 3.**

| | **Theoretical Yield of Quaternary Isomer in Product (mol%)** | |
|---|---|---|
| **Monolefin Vinylidene Content (mol %)** | **54%** | **70%** |
| **50 %** | 27 | 35 |
| **60 %** | 32 | 42 |
| **65 %** | 35 | 45 |

## Claims

1. An alkylaromatic composition comprising:
an aromatic moiety other than unsubstituted naphthalene; and
an alkyl moiety having a carbon atom number in the range between 16 to 40, wherein said alkyl moiety is attached to said aromatic moiety such that at least 25 mol% of the benzylic carbons are quaternary.

2. The alkylaromatic composition of claim 1, wherein at least 35 mol%, preferably at least 70 mol %, of the benzylic carbons are quaternary.

3. The alkylaromatic composition of claim 1, wherein said aromatic moiety is toluene and optionally said composition has an oxidative stability, as measured by ASTM D2272, of greater than 30 minutes.

4. The alkylaromatic composition of claim 1, wherein said aromatic moiety is benzene and optionally said composition has an oxidative stability, as measure by ASTM D2272, of greater than 20 minutes.

5. The alkylaromatic composition of claim 1, wherein said composition has a pour point of less than or equal to -35°C, preferably less than or equal to -50°C.

6. A process for the preparation of an alkylaromatic compound comprising: contacting at least one aromatic moiety and a mono-olefin having a carbon atom number in the range between 16 to 40 in the presence of an acidic alkylation catalyst under alkylation conditions, wherein at least 50 mol% of the mono-olefin comprises a vinylidenyl structure, and thereby producing said alkylaromatic compound having at least 25 mol% of benzylic carbons that are quaternary.

7. The process according to claim 6, further comprising: separating and recovering said alkylaromatic compound.

8. The process according to claim 6, wherein said alkylaromatic compound has at least 65 mol% of benzylic carbons that are quaternary.

9. The process according to claim 6, wherein said acidic alkylation catalyst is chosen from zeolite catalysts, MCM-22, MCM-57, MCM-36, MCM-49, MCM-56, ITQ-1, and ITQ-3, or is a Friedel Craft catalyst chosen from BF₃, promoted BF₃, AlCl₃, SnCl₄, FeCl₃, and ZnCl₂.

10. The alkylaromatic composition of claim 1 wherein said aromatic moiety is chosen from benzene, toluene, xylenes, ethylbenzene, diphenyl sulfide, diphenyl oxide, and mixtures thereof.

11. The alkylaromatic composition of claim 1 wherein said aromatic moiety is chosen from substituted or unsubstituted benzene, substituted naphthalene, substituted or unsubstituted furan, substituted or unsubstituted thiophene, substituted or unsubstituted anthracene, substituted or unsubstituted phenanthrene, substituted or unsubstituted pyrole, substituted or unsubstituted indole, substituted or unsubstituted benzothiophene, substituted or unsubstituted dibenzothiophene, substituted or unsubstituted benzofuran, substituted or unsubstituted dibenzofuran, substituted or unsubstituted phenoxanthiin, substituted or unsubstituted thianthrene, substituted or unsubstituted biphenyl, substituted or unsubstituted pyrene, bisphenol A, bisphenol sulfide, anisole, thioanisole, diphenyl oxide, diphenyl sulfide, diphenylmethane, and mixtures thereof.

12. The alkylaromatic composition of claim 1, wherein said aromatic moiety is chosen from toluene, o-, m- or p-xylene, hydroxybenzene, methoxy or ethoxybenzene, thioanisole, diphenylether, diphenylmethane, diphenyl sulfide, methylnaphthalene, methoxynaphthalene, ethoxynaphthalene, methylnaphthyl sulfide, ethyl naphthylsulfide, bisphenol-A, bisphenol sulfide and mixtures thereof.

13. The alkylaromatic composition of claim 1 or the process according to claim 6, wherein said mono-olefin has a carbon atom number in the range between 16 to 24.

14. The process according to claim 6, wherein said mono-olefin is derived from alkyl aluminum catalysts.

15. The process according to claim 14, wherein said alkyl aluminum catalyst is triisobutyl aluminum.

16. The process according to of claim 6, wherein said mono-olefin is derived from a metallocene-catalyzed alpha-olefin polymerization process.

17. The process according to claim 6, wherein said mono-olefin is derived from a vinylidene with a carbon atom number less than 40.

18. The process according to claim 17, wherein said vinylidene is chosen from 2-hexyl-1-decene, 2-octyl-1-dodecene, or 2-decyl-1-tetradecene, and mixtures thereof.

19. The process according to claim 6, wherein at least 65 mol% of the mono-olefin comprises a vinylidenyl structure.

20. The process according to claim 6, wherein said aromatic moiety is chosen from benzene, toluene, xylenes, ethylbenzene, naphthalene, diphenyl sulfide, diphenyl oxide, and mixtures thereof.

21. The process according to claim 6, wherein said aromatic moiety is chosen from substituted or unsubstituted benzene, substituted or unsubstituted naphthalene, substituted or unsubstituted furan, substituted or unsubstituted thiophene, substituted or unsubstituted anthracene, substituted or unsubstituted phenanthrene, substituted or unsubstituted pyrole, substituted or unsubstituted indole, substituted or unsubstituted benzothiophene, substituted or unsubstituted dibenzothiophene, substituted or unsubstituted benzofuran, substituted or unsubstituted dibenzofuran, substituted or unsubstituted phenoxanthiin, substituted or unsubstituted thianthrene, substituted or unsubstituted biphenyl, substituted or unsubstituted pyrene, bisphenol A, bisphenol sulfide, anisole, thioanisole, diphenyl oxide, diphenyl sulfide, diphenylmethane, and mixtures thereof.

22. The process according to claim 6, wherein said aromatic moiety is chosen from toluene, o-, m- or p-xylene, hydroxybenzene, methoxy or ethoxybenzene, thioanisole, diphenylether, diphenylmethane, diphenyl sulfide, naphthalene, methylnaphthalene, methoxynaphthalene, ethoxynaphthalene, methylnapthyl sulfide, ethyl naphthylsulfide, bisphenol-A, bisphenol sulfide and mixtures thereof.

## Patentansprüche

1. Alkylaromatische Zusammensetzung, die
eine von unsubstituiertem Naphthalin verschiedene aromatische Einheit und
eine Alkyleinheit mit einer Kohlenstoffatomanzahl im Bereich zwischen 16 und 40, wobei die Alkyleinheit so an die aromatische Einheit gebunden ist, dass mindestens 25 Mol% der benzylischen Kohlenstoffe quartär sind,
enthält.

2. Alkylaromatische Zusammensetzung nach Anspruch 1, bei der mindestens 35 Mol%, vorzugsweise mindestens 70 Mol% der benzylischen Kohlenstoffe quartär sind.

3. Alkylaromatische Zusammensetzung nach Anspruch 1, bei der die aromatische Einheit Toluol ist und die Zusammensetzung gegebenenfalls eine Oxidationsstabilität, gemessen durch ASTM D2272, von mehr als 30 Minuten aufweist.

4. Alkylaromatische Zusammensetzung nach Anspruch 1, bei der die aromatische Einheit Benzol ist und die Zusammensetzung gegebenenfalls eine Oxidationsstabilität, gemessen durch ASTM D2272, von mehr als 20 Minuten aufweist.

5. Alkylaromatische Zusammensetzung nach Anspruch 1, wobei die Zusammensetzung einen Stockpunkt von weniger als oder gleich -35°C, vorzugsweise weniger als oder gleich -50°C aufweist.

6. Verfahren zur Herstellung einer alkylaromatischen Verbindung, bei dem mindestens eine alkylaromatische Einheit und ein Monoolefin mit einer Kohlenstoffatomanzahl im Bereich zwischen 16 und 40 in Gegenwart eines sauren Alkylierungskatalysators unter Alkylierungsbedingungen in Kontakt gebracht werden, wobei mindestens 50 Mol% des Monoolefins eine Vinylidenylstruktur aufweist und dadurch die alkylaromatische Verbindung erzeugt wird, die mindestens 25 Mol% benzylische Kohlenstoffe aufweist, welche quartär sind.

7. Verfahren nach Anspruch 6, bei dem ferner die alkylaromatische Verbindung getrennt und gewonnen wird.

8. Verfahren nach Anspruch 6, bei dem die alkylaromatische Verbindung mindestens 65 Mol% benzylische Kohlenstoffe aufweist, die quärtär sind.

9. Verfahren nach Anspruch 6, bei dem der saure Alkylierungskatalysator ausgewählt ist aus Zeolithkatalysatoren, MCM-22, MCM-57, MCM-36, MCM-49, MCM-56, ITQ-1 und ITQ-3 oder ein Friedel-Craft-Katalysator ausgewählt aus BF₃, BF₃ mit Promotor, AlCl₃, SnCl₄, FeCl₃ und ZnCl₂ ist.

10. Alkylaromatische Zusammensetzung nach Anspruch 1, bei der die aromatische Einheit ausgewählt ist aus Benzol, Toluol, Xylolen, Ethylbenzol, Diphenylsulfid, Diphenyloxid und deren Mischungen.

11. Alkylaromatische Zusammensetzung nach Anspruch 1, bei der die aromatische Einheit ausgewählt ist aus substituiertem oder unsubstituiertem Benzol, substituiertem Naphthalin, substituiertem oder unsubstituiertem Furan, substituiertem oder unsubstituiertem Tiophen, substituiertem oder unsubstituiertem Anthracen, substituiertem oder unsubstituiertem Phenanthren, substituiertem oder unsubstituiertem Pyrol, substituiertem oder unsubstituiertem Indol, substituiertem oder unsubstituiertem Benzothiophen, substituiertem oder unsubstituiertem Dibenzothiophen, substituiertem oder unsubstituiertem Benzofuran, substituiertem oder unsubstituiertem Dibenzofuran, substituiertem oder unsubstituiertem Phenoxanthiin, substituiertem oder unsubstituiertem Thianthren, substituiertem oder unsubstituiertem Biphenyl, substituiertem oder unsubstituiertem Pyren, Bisphenol-A, Bisphenolsulfid, Anisol, Thioanisol, Diphenyloxid, Diphenylsulfid, Diphenylmethan und deren Mischungen.

12. Alkylaromatische Zusammensetzung nach Anspruch 1, bei der die aromatische Einheit ausgewählt ist aus Toluol, o-, m- oder p-Xylol, Hydroxybenzol, Methoxy- oder Ethoxybenzol, Thioanisol, Diphenylether, Diphenylmethan, Diphenylsulfid, Methylnaphthalin, Methoxynaphthalin, Ethoxynaphtalin, Methylnapthylsulfid, Ethylnaphtylsulfid, Bisphenol-A, Bisphenolsulfid und deren Mischungen.

13. Alkylaromatische Zusammensetzung nach Anspruch 1 oder Verfahren nach Anspruch 6, bei dem das Monoolefin eine Kohlenstoffatomanzahl im Bereich zwischen 16 und 24 aufweist.

14. Verfahren nach Anspruch 6, bei dem das Monoolefin von Alkylaluminiumkatalysatoren abgeleitet ist.

15. Verfahren nach Anspruch 14, bei dem der Alkylaluminiumkatalysator Triisobutylalumnium ist.

16. Verfahren nach Anspruch 6, bei dem das Monoolefin aus einem Mellocen-katalysiertem Verfahren zur Polymerisation von alpha-Olefinen abgeleitet ist.

17. Verfahren nach Anspruch 6, bei dem das Monoolefin aus einem Vinyliden mit einer Kohlenstoffatomanzahl von weniger als 40 abgeleitet ist.

18. Verfahren nach Anspruch 17, bei dem das Vinyliden ausgewählt ist aus 2-Hexyl-1-decen, 2-Octyl-1-dodecen oder 2-Decyl-1-teteradecen und deren Mischungen.

19. Verfahren nach Anspruch 6, bei dem mindestens 65 Mol% des Monoolefins eine Vinylidenylstruktur umfassen.

20. Verfahren nach Anspruch 6, bei dem die aromatische Einheit ausgewählt ist aus Benzol, Toluol, Xylolen, Ethylbenzol, Diphenylsulfid, Diphenyloxid und deren Mischungen.

21. Verfahren nach Anspruch 6, bei dem die aromatische Einheit ausgewählt ist aus substituiertem oder unsubstituiertem Benzol, substituiertem oder unsubstituiertem Naphthalin, substituiertem oder unsubstituiertem Furan, substituiertem oder unsubstituiertem Tiophen, substituiertem oder unsubstituiertem Anthracen, substituiertem oder unsubstituiertem Phenanthren, substituiertem oder unsubstituiertem Pyrol, substituiertem oder unsubstituiertem Indol, substituiertem oder unsubstituiertem Benzothiophen, substituiertem oder unsubstituiertem Dibenzothiophen, substituiertem oder
unsubstituiertem Benzofuran, substituiertem oder unsubstituiertem Dibenzofuran, substituiertem oder unsubstituiertem Phenoxanthiin, substituiertem oder unsubstituiertem Thianthren, substituiertem oder unsubstituiertem Biphenyl, substituiertem oder unsubstituiertem Pyren, Bisphenol-A, Bisphenolsulfid, Anisol, Thioanisol, Diphenyloxid, Diphenylsulfid, Diphenylmethan und deren Mischungen.

22. Verfahren nach Anspruch 6, bei dem die aromatische Einheit ausgewählt ist aus Toluol, o-, m- oder p-Xylol, Hydroxybenzol, Methoxy- oder Ethoxybenzol, Thioanisol, Diphenylether, Diphenylmethan, Diphenylsulfid, Naphthalin, Methylnaphthalin, Methoxynaphthalin, Ethoxynaphtalin, Methylnapthylsulfid, Ethylnaphtylsulfid, Bisphenol-A, Bisphenolsulfid und deren Mischungen.

## Revendications

1. Composition alkylaromatique comprenant :
un groupement aromatique autre que naphtalène non substitué ; et
un groupement alkyle comportant un nombre d'atomes de carbone dans la fourchette entre 16 et 40, ledit groupement alkyle étant fixé audit groupement aromatique de telle sorte qu'au moins 25 % en moles des atomes de carbone benzyliques soient quaternaires.

2. Composition alkylaromatique selon la revendication 1, dans laquelle au moins 35 % en moles, de préférence au moins 70 % en moles, des atomes de carbone benzyliques sont quaternaires.

3. Composition alkylaromatique selon la revendication 1, dans laquelle ledit groupement aromatique est le toluène et éventuellement ladite composition possède une stabilité à l'oxydation, mesurée par ASTM D2272, de plus de 30 minutes.

4. Composition alkylaromatique selon la revendication 1, dans laquelle ledit groupement aromatique est le benzène et éventuellement ladite composition possède une stabilité à l'oxydation, mesurée par ASTM D2272, de plus de 20 minutes.

5. Composition alkylaromatique selon la revendication 1, dans laquelle ladite composition possède un point d'écoulement inférieur ou égal à -35°C, de préférence inférieur ou égal à -50°C.

6. Procédé de préparation d'un composé alkylaromatique comprenant : la mise en contact d'au moins un groupement aromatique et d'une mono-oléfine comportant un nombre d'atomes de carbone dans la fourchette entre 16 à 40 en présence d'un catalyseur d'alkylation acide dans des conditions d'alkylation, dans lequel au moins 50 % en moles de la mono-oléfine comprennent une structure vinylidényle, et permettant ainsi de produire ledit composé alkylaromatique comportant au moins 25 % en moles d'atomes de carbone benzyliques qui sont quaternaires.

7. Procédé selon la revendication 6, comprenant en outre : la séparation et la récupération dudit composé alkylaromatique.

8. Procédé selon la revendication 6, dans lequel ledit composé alkylaromatique possède au moins 65 % en moles d'atomes de carbone benzyliques qui sont quaternaires.

9. Procédé selon la revendication 6, dans lequel ledit catalyseur d'alkylation acide est choisi parmi les catalyseurs zéolithiques, MCM-22, MCM-57, MCM-36, MCM-49, MCM-56, ITQ-1 et ITQ-3, ou est un catalyseur de Friedel Craft choisi parmi BF₃, BF₃ activé, AlCl₃, SnCl₄, FeCl₃ et ZnCl₂.

10. Composition alkylaromatique selon la revendication 1 dans laquelle ledit groupement aromatique est choisi parmi le benzène, le toluène, les xylènes, l'éthyl-benzène, le sulfure de diphényle, l'oxyde de diphényle, et des mélanges de ceux-ci.

11. Composition alkylaromatique selon la revendication 1 dans laquelle ledit groupement aromatique est choisi parmi le benzène substitué ou non substitué, le naphtalène substitué, le furane substitué ou non substitué, le thiophène substitué ou non substitué, l'anthracène substitué ou non substitué, le phénanthrène substitué ou non substitué, le pyrole substitué ou non substitué, l'indole substitué ou non substitué, le benzothiophène substitué ou non substitué, le dibenzothiophène substitué ou non substitué, le benzofurane substitué ou non substitué, le dibenzofurane substitué ou non substitué, la phénoxanthine substituée ou non substituée, le thianthrène substitué ou non substitué, le biphényle substitué ou non substitué, le pyrène substitué ou non substitué, le bisphénol A, le sulfure de bisphénol, l'anisole, le thioanisole, l'oxyde de diphényle, le sulfure de diphényle, le diphénylméthane, et des mélanges de ceux-ci.

12. Composition alkylaromatique selon la revendication 1, dans laquelle ledit groupement aromatique est choisi parmi le toluène, l'o-, m- ou p-xylène, l'hydroxybenzène, le méthoxy ou éthoxybenzène, le thioanisole, le diphényléther, le diphénylméthane, le sulfure de diphényle, le méthylnaphtalène, le méthoxynaphtalène, l'éthoxynaphtalène, le sulfure de méthylnaphtyle, le sulfure d'éthylnaphtyle, le bisphénol-A, le sulfure de bisphénol et des mélanges de ceux-ci.

13. Composition alkylaromatique selon la revendication 1 ou procédé selon la revendication 6, dans lequel ladite mono-oléfine possède un nombre d'atomes de carbone dans la fourchette entre 16 à 24.

14. Procédé selon la revendication 6, dans lequel ladite mono-oléfine est dérivée de catalyseurs de type alkyl-aluminium.

15. Procédé selon la revendication 14, dans lequel ledit catalyseur de type alkyl-aluminium est le triisobutyl-aluminium.

16. Procédé selon la revendication 6, dans lequel ladite mono-oléfine est dérivée d'un procédé de polymérisation d'alpha-oléfine catalysée par un métallocène.

17. Procédé selon la revendication 6, dans lequel ladite mono-oléfine est dérivée d'un vinylidène ayant un nombre d'atomes de carbone inférieur à 40.

18. Procédé selon la revendication 17, dans lequel ledit vinylidène est choisi parmi le 2-hexyl-1-décène, le 2-octyl-1-dodécène ou le 2-décyl-1-tétradécène, et des mélanges de ceux-ci.

19. Procédé selon la revendication 6, dans lequel au moins 65 % en moles de la mono-oléfine comprend une structure vinylidényle.

20. Procédé selon la revendication 6, dans lequel ledit groupement aromatique est choisi parmi le benzène, le toluène, les xylènes, l'éthylbenzène, le naphtalène, le sulfure de diphényle, l'oxyde de diphényle, et des mélanges de ceux-ci.

21. Procédé selon la revendication 6, dans lequel ledit groupement aromatique est choisi parmi le benzène substitué ou non substitué, le naphtalène substitué ou non substitué, le furane substitué ou non substitué, le thiophène substitué ou non substitué, l'anthracène substitué ou non substitué, le phénanthrène substitué ou non substitué, le pyrole substitué ou non substitué, l'indole substitué ou non substitué, le benzothiophène substitué ou non substitué, le dibenzothiophène substitué ou non substitué, le benzofurane substitué ou non substitué, le dibenzofurane substitué ou non substitué, la phénoxanthine substituée ou non substituée, le thianthrène substitué ou non substitué, le biphényle substitué ou non substitué, le pyrène substitué ou non substitué, le bisphénol A, le sulfure de bisphénol, l'anisole, le thioanisole, l'oxyde de diphényle, le sulfure de diphényle, le diphénylméthane, et des mélanges de ceux-ci.

22. Procédé selon la revendication 6, dans lequel ledit groupement aromatique est choisi parmi le toluène, l'o-, m- ou p-xylène, l'hydroxybenzène, le méthoxy ou éthoxybenzène, le thioanisole, le diphényléther, le diphénylméthane, le sulfure de diphényle, le naphtalène, le méthylnaphtalène, le méthoxynaphtalène, l'éthoxynaphtalène, le sulfure de méthylnaphtyle, le sulfure d'éthylnaphtyle, le bisphénol-A, le sulfure de bisphénol et des mélanges de ceux-ci.
